

Patented Apr. 9, 1929.

1,708,058

# UNITED STATES PATENT OFFICE.

PRESTON C. GOSS, OF MUNCIE, INDIANA.

## LUBRICATING MIXTURE AND PROCESS OF MAKING SAME.

No Drawing.

Application filed February 7, 1927. Serial No. 166,588.

My invention relates to improvements in lubricating mixtures, and the process of making the same.

An object of my invention is to provide a lubricating mixture which will obviate certain of the disadvantages that attach to the mineral oils now in use. One of these disadvantages is that under certain conditions there is not the proper adhesion of the oil to the metal surface and this results in excessive wear because of the fact that the lubricating fluid has not sufficiently covered the surface. My invention is designed to provide a lubricant which will adhere to the metal and which will cause the lubricant to coat it so that the friction is greatly reduced.

A further object of the invention is to provide a lubricating mixture which can be used in connection with internal combustion engines and which tends to seal the space between the piston rings and the cylinder so completely that gasoline is prevented from passing the piston and from diluting the oil in the crank-case.

25 A further object is to provide a process by means of which the lubricating mixture is prepared.

Other objects and advantages will appear in the following specification, and the novel features of the invention will be particularly pointed out in the appended claims.

In carrying out my invention, I make use of the inner mucilaginous bark of the *Ulmus fulva* (slippery elm). This bark is ground or shredded when dry or partially so and is enclosed in a bag of muslin or similar cloth and then is immersed in water, preferably kept at 80° F. and allowed to stand for six hours.

40 The bag with its water fluid contents is then lifted from the tank or receptacle in which it has been immersed and the surplus water is allowed to drain from it. The bag is afterwards put in a press and the liquid extract is forced out. The pressure is gauged so as not to press out any solids.

The expressed mucilaginous liquid is now mixed with a good mineral lubricating oil of a petroleum base of medium grade. The proportions are one part of the expressed mucilaginous liquid to five parts of the mineral lubricating oil. The mixture is now put into a mechanical mixer and is agitated from five to fifteen minutes or until the mixture has the appearance of a smooth cream and is free from any small lumps and is of a homogeneous texture and of a uniform color.

The mixture which is in the nature of an emulsion is now placed in a receptacle and allowed to stand for some time, preferably for twelve hours, during which time any solids which may have been in the mixture have been precipitated and any unemulsified water will have also passed to the bottom. The remaining portion of the mixture is decanted; that is to say, that portion above the sediment and water is drawn off and this constitutes the lubricating emulsion which forms the subject of the present invention. This emulsion I will call "A".

The emulsion "A" can now be mixed with any suitable mineral lubricating oil of a petroleum base in any desired proportions for use. I have found that good proportions for use are one part of the emulsion "A" to eight parts of oil for a light lubricant, one to seven for medium, and one to six for a heavy lubricant.

In trying out this lubricant in practice I have found that it tends to seal the space between the piston rings and the cylinder wall in an internal combustion engine, thereby preventing the flow of gasoline into the crank-case.

While I have spoken of the use of the mixture for internal combustion engines, it will be understood that any lubricating oil other than mineral oil of a petroleum base and hard grease may be prepared with mucilaginous liquid from the inner bark of the *Ulmus fulva* (slippery elm). This latter oil and grease is treated in the same manner as the mineral oil of a petroleum base and in every instance the adhesion of the oil or grease to the part to be lubricated appears to be increased and thus the lubricating effect is increased since it holds the oil on the part to be lubricated or causes it to cling to the surface, thus greatly reducing wear, and, in the instance given above, forming a seal in the internal combustion engine for preventing the passage of gasoline.

I claim:

1. A lubricating emulsion, consisting of a mineral lubricating oil and an aqueous extract of the *Ulmus fulva* in proportions of substantially five parts by volume of the oil and one part by volume of the extract.
2. The herein described process of making a lubricating emulsion, which consists in mixing with a mineral lubricating oil an aqueous extract of the inner bark of the *Ulmus fulva*, permitting the mixture to settle, and separat-

ing the lighter fluid emulsion from the sediment and unemulsified water.

3. The herein described process of making a lubricating emulsion, which consists in mixing with a mineral lubricating oil an aqueous extract of the inner bark of the *Ulmus fulva* in proportions of substantially five parts by volume of the oil and one part by volume of the extract, permitting the mixture to settle, separating the lighter fluid emulsion from the sediment and unemulsified water, and mixing with the emulsion a mineral lubricating oil in proportions of substantially one part by volume of the extract and seven parts by volume of the mineral lubricating oil.

4. A lubricating emulsion, consisting of a

mineral lubricating oil having its particles intimately mixed with particles of an aqueous extract of the inner bark of the *Ulmus fulva*. 20

5. A lubricating emulsion, consisting of a mineral lubricating oil and an aqueous extract of the inner bark of the *Ulmus fulva* in proportions of substantially five parts by volume of the oil and one part by volume of the 25 extract, and one part by volume of the emulsion and seven parts by volume of a mineral lubricating oil.

6. A lubricating emulsion, consisting of a mineral lubricating oil of a petroleum base and an aqueous extract of the inner bark of 30 slippery elm.

PRESTON C. GOSS.